

# UNITED STATES PATENT OFFICE.

FRANK A. FAHRENWALD, OF CLEVELAND, OHIO.

## FIREARM AND ALLOY FOR MAKING SAME.

1,346,188.

Specification of Letters Patent. Patented July 13, 1920.

No Drawing.

Application filed August 25, 1919. Serial No. 319,822.

To all whom it may concern:

Be it known that I, FRANK A. FAHRENWALD, a citizen of the United States, residing at Cleveland, in the county of Cuyahoga and State of Ohio, have invented a certain new and useful Improvement in Firearms and Alloys for Making Same, of which the following is a full, clear, and exact description.

10 This invention relates to firearms and ordnance and has for its particular object the provision of a metallic alloy for use in the construction of the same which shall be more resistant to corrosion by the combustion products of the explosive, as well as less corroded by atmospheric conditions, salt solutions (such as sea water or sweaty hands), than anything previously used for the purpose, as well as having sufficient mechanical strength to endure the strains to which such devices are subjected, and at the same time being sufficiently soft and workable for manufacturing purposes.

It is well known that powder gases, particularly those of the present day smokeless and high explosive powders, are extremely corrosive to steel barrels so that the latter become rapidly etched and pitted. This circumstance has greatly shortened the life 25 of sporting arms and has rendered very onerous the maintenance of military arms of all calibers, since not only have the metals heretofore employed suffered greatly by the instant erosion of the hot gases but the powder residues are of an equally great corrosiveness and cannot be removed by mere physical means nor even by a single application of chemicals. Unless such a firearm be cleaned within at least an hour after each 30 shot, the barrel interior becomes noticeably etched, and even a few very small pits seriously impairs the accuracy of the gun. Likewise the exteriors of the barrels and the surfaces of the operating mechanism become 35 rapidly corroded by atmospheric influences and skin contact unless frequently oiled. Furthermore, most high velocity rifle bullets used at the present day are jacketed with some alloy which will keep the lead from 40 melting and will engage the rifling properly. Most of these jacket materials possess such an affinity for the iron of which rifle barrels have heretofore been made as to alloy therewith under the influence of high temperature, velocity and pressure, thus producing

the phenomenon known as "metal fouling," which means a slow accretion inside the barrel of substance taken from the bullets, which always interferes seriously with the accuracy, and frequently leads to bursting 60 of the barrel.

Numerous alloys have heretofore been known which would resist the chemical action to the necessary extent, (such as alloys of platinum, gold-palladium, and the like precious metals), but the physical requirements of firearms metal are also peculiarly exacting since it must be sufficiently soft and uniform to permit of ready boring and rifling of the barrel and fashioning of 70 the operating mechanism, and yet possess sufficient toughness and mechanical strength to resist the explosion pressures and the mishaps to which such devices are necessarily subjected in use. 75

The objects of my invention are, therefore, the provision of an alloy for the purposes stated having the requisite chemical resistivity coupled with the necessary physical strength; the provision of an alloy which 80 shall not be subject to "metal fouling;" the provision of an alloy which can be readily forged, machined and worked into shape; the provision of an alloy of reasonably low intrinsic value and containing only readily 85 available ingredients; the provision of an alloy which can be made by a simple and workable process; while further objects and advantages of my invention will become apparent as the description proceeds. 90

My improved alloy consists essentially of one or more iron group metals combined with one or more chromium group metals. Carbon and silicon may be present in case their quantities are small, say .5% or less; 95 a small amount of manganese is preferably employed because of its value in scavenging oxygen and sulfur and because of the fact that better castings are secured with its use. The tensile strength of the alloy can be increased slightly by the addition of a small amount of copper, tantalum, vanadium, zirconium, or titanium, although the strength of the simpler alloy is sufficiently great so that no particular advantage is secured by 100 their use. All these minor modifications fall within the scope of my generic idea and the presence or absence of these additional substances does not modify my invention. 105

As examples of alloys which embody my 110

invention, I will instance the following, the first column indicating the preferred composition within that group and the parentheses indicating the permissible variations.

|    |                           |                                                  |         |
|----|---------------------------|--------------------------------------------------|---------|
| 5  | Nickel                    | 55                                               | (10-55) |
| a  | Chromium                  | 15                                               | (8-20)  |
|    | Iron                      | 30                                               | (82-25) |
| b  | Iron                      | 75                                               | (60-90) |
|    | Chromium                  | 25                                               | (10-40) |
| 10 | Nickel                    | 85                                               | (70-95) |
| c  | Chromium                  | 15                                               | (5-30)  |
| d  | Nickel                    | 90                                               | (85-95) |
|    | Tungsten or molybdenum    | 10                                               | (5-15)  |
| 15 | Iron                      | 90                                               | (80-95) |
| e  | Tungsten or molybdenum    | 10                                               | (5-20)  |
|    | Any two iron group metals | 90                                               | (75-95) |
| f  | Tungsten or molybdenum    | 10                                               | (5-25)  |
|    | Any two iron group metals | 70-90                                            |         |
| 20 | g                         | Chromium and one other metal from chromium group | 10-30   |
|    | Iron or nickel            | 70-90                                            |         |
| h  | Cobalt                    | 5-20                                             |         |
|    | Chromium or tungsten      | 5-25                                             |         |

25 It will be understood that the foregoing formulas are not intended to include all the ingredients present in the alloys, since small amounts of carbon, silicon, and manganese will almost always be present, and small 30 quantities of certain additional metals may sometimes be added such as copper etc. as has already been suggested. It is only necessary that the percentage of carbon and silicon be kept sufficiently low, such as .5% 35 or less of each, to prevent the metal from being too hard to work, and that sulfur and phosphorus be avoided.

The requirements of different guns are so various, especially when low intrinsic 40 value is considered as a requirement, that no one alloy can be denominated a preferred species for all uses. Thus the alloy of group *a* containing nickel 55%, chromium 30% and iron 15%, exhibits every 45 desirable chemical and mechanical property in the highest degree. It can be made with comparative ease in the electric furnace or by the alumino-thermic method it makes a good casting, can readily be forged or rolled 50 at a bright red heat, and can be bored, turned, rifled, and shaped without difficulty. The gases and residues of smokeless powder do not etch it even in days 55 of neglect, rain does not rust it, and polished barrels buried in the ground for weeks exhibit only a slight superficial tarnish which can be wiped off with the hand. Bullet jackets of iron, nickel, or their alloys do not foul it, and its tensile strength is so 60 high that it compares well with the steels ordinarily used. This alloy is good enough for almost every purpose but can be only slightly improved by the addition of a little molybdenum or tungsten which will still 65 further increase the chemical resistivity.

The only drawback is that it is unnecessarily good for some purposes. For example in a .22 caliber boy's rifle, the bursting strains are so small as to be withstood by any metal which is strong enough to resist 70 the mechanical shocks of use. Other and cheaper alloys can be found which will possess chemical resistivity without such an excess of mechanical strength.

For example the percentage of iron can 75 be increased as shown under *a* or the nickel entirely eliminated, as shown under *b*; in this case the permissible chromium content becomes much higher, the hardening effect of nickel thereon being removed. The addition of tungsten or molybdenum to the 80 alloy shown at *b* increases both its strength and its chemical resistivity.

The substitution of nickel for iron in *b* gives *c* which is superior in the same proportion that nickel is superior to iron in 85 chemical resistivity. Owing to the hardening effect of chromium thereon the proportion of the latter is decreased. It will be understood that cobalt can be employed in 90 substitution for iron or nickel or in addition thereto, although no advantage in its use offsets its high price.

If tungsten or molybdenum be employed 95 in place of chromium in *c*, I secure the alloy shown at *d* which is also hard, strong and chemically resistant; or if the chromium in *b* is replaced by tungsten or molybdenum I secure the alloy shown at *e* which is also of value for firearms. In these cases the amount 100 of the tungsten-like metal is decreased owing to its hardening effect.

I find the ternary alloys better than the binary alloys for this purpose, wherefore I prefer the compositions shown in *a*, *f*, or *g*, 105 or one made by adding tungsten or molybdenum to *b* or *c*. In fact for some purposes the very best alloy appears to be a quaternary as produced by adding tungsten or molybdenum to *a* or chromium to *f*. I do, 110 however, find that the essential elements are those contained in the iron and chromium groups of the periodic table and that at least one metal from each group should be used; also the chromium group metal should occur 115 to an amount of at least about 5% and should not go above about 25% unless the iron group metal be iron alone and the chromium group metal be chromium alone in which case the percentage of the latter 120 can be increased up to about 40% without rendering the alloy too hard to work.

It will be understood that while my improved alloy is specially devised for manually portable arms such as rifles and shot- 125 guns it is equally good for pocket devices such as revolvers or for ordnance of large sizes; that the barrels can be made from a single homogeneous piece of the material, or that a composite ingot may be made, or a 130

built up barrel employing my improved alloy as a lining; that my alloy can be used for lock mechanisms equally with the barrels; and that I desire my claims taken in the 5 broadest sense that their language will support.

Having thus described my invention what I claim is:—

1. A firearm barrel made from an alloy of 10 one or more iron group metals combined with one or more chromium group metals.

2. A firearm barrel made from an alloy of 15 one or more iron group metals combined with one or more chromium group metals, the latter being present to an amount of at least 5%.

3. A firearm barrel made from an alloy of two iron group metals together with at least one chromium group metal.

20 4. A firearm barrel made from an alloy of two iron group metals together with chromium and another metal from the chromium group.

5. A firearm barrel made from an alloy 25 containing at least 5% of chromium, at least 5% of nickel and not more than 90% of iron.

6. A firearm barrel made from an alloy containing between 5% and 25% of one or 30 more metals of the chromium group combined with metals of the iron group, not more than 90% of the whole alloy being iron.

7. A firearm having a barrel composed of 35 or lined with an alloy of iron, nickel and chromium wherein the chromium and nickel each comprises not less than about 10% of the whole.

8. A firearm having a barrel composed of 40 or lined with an alloy of iron, nickel and chromium wherein the iron constitutes not over about 60%, the nickel at least 20% and the balance mostly chromium.

9. A firearm having a barrel composed of 45 or lined with an alloy of iron, nickel and chromium, wherein the iron constitutes not over about 40%, chromium between 15% and 20% and the balance mostly nickel.

10. A firearm having a barrel composed of 50 or lined with an alloy of iron, nickel and chromium wherein the iron constitutes about 30%, the chromium between 15% and 20% and the balance mostly nickel.

11. A firearm having parts made of an alloy containing less than about 80% of iron 55 alloyed with more than 10% of nickel and at least 8% of chromium.

12. A firearm having parts made of an alloy comprising between 8% and 20% chromium, together with between about 25% 60 and about 80% iron, the balance being principally nickel.

13. A firearm having parts made of an alloy whose principal ingredients are iron, nickel and chromium, these ingredients occurring in the relative proportions of iron 65

between 25% and 80%, nickel between 20% and 55% and chromium between 8% and 20%.

14. A firearm having a barrel made of an alloy containing less than 80% of iron combined with more than 10% of chromium, the balance consisting largely of other metals from the iron and chromium groups. 70

15. A firearm having parts made of an alloy containing less than 90% of iron combined with at least 5% of a metal from the chromium group, any remainder of the alloy consisting principally of other metals from the iron and chromium groups. 75

16. A firearm having a barrel composed of or lined with an alloy containing between 30% and 90% of iron, and at least 10% of chromium, any remainder of the alloy consisting principally of nickel. 80

17. A firearm having a barrel composed of or lined with an alloy containing not over 90% of iron and not less than 10% of chromium. 85

18. A firearm having a barrel composed of or lined with an alloy containing a pre- 90 ponderance of iron group metals together with from 5% to 20% of metals below chromium in the chromium group.

19. A firearm having a barrel composed of, or lined with, an alloy containing a plurality of iron group metals to a total of from 75% to 95%, the balance being chromium group metals. 95

20. A firearm having a barrel composed of or lined with an alloy containing a plurality of iron group metals to a total proportion of between 75% and 90% combined with chromium group metals, chromium itself constituting at least one-half of the balance. 100

21. A firearm barrel made of an alloy containing iron combined with at least ten per cent. of one or more of the metals nickel and chromium. 105

22. A firearm barrel made of an alloy containing between about twenty-five per cent. and about ninety per cent. of iron, the balance being principally nickel and chromium and carbon being present to an amount not greater than two tenths of one 110 per cent. 115

23. A firearm barrel made of an alloy characterized by the presence of more than ten per cent. of one or both of the metals nickel and chromium. 120

24. A firearm barrel made of an alloy containing one or more iron group metals alloyed with such an amount of chromium that the total amount of non-ferrous metal in the alloy shall constitute at least about 125 ten per cent. of the whole.

25. A firearm barrel made of an alloy of one or more iron group metals with chromium, the amount of chromium being such as together with the non-ferrous metal 130

of the alloy shall constitute at least ten per cent. of the whole.

26. A firearm barrel made of an alloy consisting essentially of iron with either or both nickel and (or) chromium, the highest limit of chromium being about twenty-five per cent. and the highest limit of iron

being about ninety per cent. and the lowest limit of nickel or chromium or some combination of the two being not less than 10 about ten per cent.

In testimony whereof I hereunto affix my signature.

FRANK A. FAHRENWALD.